

# UNITED STATES PATENT OFFICE.

DAVID BELAIS, OF NEW YORK, N. Y.

## PRODUCTION OF WHITE GOLD.

1,330,231.

Specification of Letters Patent. Patented Feb. 10, 1920.

No Drawing.

Application filed October 5, 1918. Serial No. 256,993.

*To all whom it may concern:*

Be it known that I, DAVID BELAIS, a citizen of the United States, and a resident of New York city, in the county and State of New York, have invented a new and useful Improvement in the Production of White Gold, of which the following is a specification.

My invention relates to the production of a substitute for platinum. The object of my invention is to produce a composition of matter known as white gold that will have the appearance of platinum and that may be used as a substitute for it, especially in the jewelry trade. It consists of the novel process and product herein described.

Platinum has always been a rare metal, and an expensive one, and in recent times it has become more and more so, until now the supply is wholly insufficient to meet the demand, and the expense has become practically prohibitive. As is well known, platinum is peculiarly well fitted for such uses, especially in the jewelry art, as the setting of diamonds, the ornamentation of watch cases, and similar articles. By my improved process I produce a white gold that has the appearance of platinum and has characteristics that fit it extremely well for use as a substitute for platinum for the setting of diamonds, the ornamentation of watch cases, and similar articles, and for other similar uses, especially in the jewelry trade.

The cost of its ingredients, and the process of producing it is relatively very small compared with that of platinum.

In my improved process I take gold, especially or preferably fine gold, nickel, preferably pure nickel, and zinc, preferably pure zinc, and fuse them together in a suitable

crucible, thoroughly mixing them together while they are thus fused. The resulting composition has the appearance of platinum and is adapted to be used as a substitute for it as already stated. It is ductile and malleable.

The matter is then prepared for the market by being rolled or hammered into plates, wires, or other forms for commercial use. It is then ready for the trade.

I use a major part of fine gold, and lesser parts of pure nickel and zinc. I have found that satisfactory results can be obtained when the fine gold is used in the proportion of about seventy-five (75) to eighty-five (85) per cent., pure nickel in the proportion of about ten (10) to eighteen (18) per cent., and pure zinc in about the proportion of two (2) to nine (9) per cent.

What I claim as new and desire to secure by Letters Patent, is:

1. As a composition of matter a white gold alloy composed of a major part of gold, and lesser proportions of nickel and zinc.

2. As a composition of matter, a white gold alloy composed of a major part of gold, a lesser proportion of nickel, and a still lesser proportion of zinc.

3. As a composition of matter, a white gold alloy composed of gold, nickel and zinc, the proportion of the gold ranging from seventy-five to eighty-five per cent., the nickel from ten to eighteen per cent., and the zinc from two to nine per cent.

4. An alloy containing a preponderating amount of gold together with relatively low percentages of nickel and zinc.

In testimony whereof I have signed my name to this specification.

DAVID BELAIS.